

March 11, 1969

J. DARIGO ET AL

3,431,612

PROCESS OF FORMING JACKETED PROJECTILES

Filed May 5, 1967

Sheet 1 of 2

Fig. 1.



Fig. 2.



Fig. 4.



Fig. 3.



Fig. 5.



Inventors:  
Julius Darigo,  
Rex E. Dickey,  
David S. Reed.

by *John H. Lewis Jr.*  
*John W. Phipps*  
*Nicholas Skovran*  
Their Attorneys

March 11, 1969

J. DARIGO ET AL

3,431,612

PROCESS OF FORMING JACKETED PROJECTILES

Filed May 5, 1967

Sheet 2 of 2

Fig. 6.



Fig. 7.



Fig. 8.



Fig. 9.



Inventors:

Julius Darigo,  
Rex E. Dickey,  
David S. Reed.

by *John H. Reeves Jr.*  
*John W. Phipps*  
*Nicholas Skouras*  
Their Attorneys

1

3,431,612  
PROCESS OF FORMING JACKETED  
PROJECTILES

Julius Darigo, Trumbull, Rex E. Dickey, Huntington, and David S. Reed, Shelton, Conn., assignors to Remington Arms Company, Inc., Bridgeport, Conn., a corporation of Delaware

Filed May 5, 1967, Ser. No. 636,495

U.S. Cl. 29—1.23

Int. Cl. B22d 19/00; B21k 21/06

8 Claims

## ABSTRACT OF THE DISCLOSURE

A method of making a small arms jacketed projectile by electrodepositing a deformable metal jacket over a softer deformable projectile core and then forming the plated projectile to its final dimensions. A modification of the process calls for forming grooves on the projectile core prior to plating so that upon plating, the grooves are filled with electrodeposited material to facilitate mushrooming of the plated projectile.

### Cross reference to related application

The present application is a division of a copending application entitled, "Process of Forming Jacketed Projectiles," Ser. No. 416,466, filed Dec. 7, 1964, now Patent No. 3,349,722, the filing date of which is claimed.

### Background of the invention

The United States patent to T. F. Werme, No. 2,336,143, issued on Dec. 7, 1943, concludes a discussion on electroplating bullets by stating that this method "... may be fairly regarded as unsatisfactory."

Werme discusses in the above-cited patent the conventional method of making jacketed projectiles in the 1941-1943 period and this method is still the conventional way of making jacketed bullets. Thus, a multiplicity of operations is necessary comprising first alternate drawings and annealings of a gilding metal jacket disc until it is formed in the shape of an elongated cup and then subsequently inserting a separately formed slug or core into the prepared jacket. In addition to the multi-operations and expensive equipment needed to make jacketed bullets under this process, the end product has certain undesirable deficiencies.

Thus, there is considerably more variation in the jacket thickness and concentricity with the conventional bullet than is experienced with electrodeposited jacketed bullets made by the present method.

Moreover, in the conventional jacketed bullets, there is no bonding between the metal cup jacket and the core so that upon impact, although the core may mushroom, the core and the jacket often become separated.

A plated bullet, made by the process explained below, and illustrated in FIGURE 1 has several important advantages over conventionally-made jacketed bullets. First, the lead core is entirely covered with a uniform thickness of copper, or other electrodepositable metal. There is no exposed soft lead nose to become damaged in handling or in use in automatic weapons.

By performing a limited amount of forming after the copper jacket is electrodeposited, a high degree of perfection in obtaining desired dimensions and shape can be achieved. In this respect, in most instances, it is important that the unplated bullet core should be approximately the same size and shape as the core in the finished plated bullet, otherwise shifting of the core inside the jacket during final forming may fracture the bond between the jacket and the lead core causing loose jackets. In some cases, the profile of the plated lead core can be changed

2

substantially while retaining the bond between the jacket and the core.

A mechanical bond is achieved between the lead core and the copper jacket which is stronger than the lead core. This results in the copper jacket remaining attached to the lead core consistently upon impacting the target, thus providing more shock impact power. The barrel tumbling electrodepositing feature assists in this mechanical bonding and further results in a very uniform and tightly inherent layer of copper being deposited on the lead core, thus insuring a more stabilized bullet.

As can be seen in FIGURE 4, there is some fingering penetration of the copper in the lead due to the surface discontinuities on the lead core into which the copper has plated. This fingering penetration of the copper in the lead core results in a mechanical bond between the lead core and the copper jacket which is stronger than the lead core. It should be appreciated that the constant tumbling of the bullets in the plating bath will result in the electrodeposited copper being impacted into the surface discontinuities of the lead core thus assisting in producing the strong bond between the core and the jacket.

The electrodeposited copper jackets are generally harder than the gilding metal jackets now in common use. Although there is an optimum desired thickness of copper plating, this thickness varies with the bullet use, the caliber of the bullet and its velocity. A thicker layer is required for mushrooming bullets, for bullets fired at high speeds and for larger caliber bullets. If the electrodeposited jacket is less than the optimum thickness for the particular mushrooming bullet caliber and velocity, the jacket will strip away from the core upon impact of the bullet. Of course, a too-heavy jacket will result in poor mushrooming qualities as well as raise the cost of making the bullet.

Additional advantages of the present barrel electrodepositing method over the conventional method mentioned above are the elimination of the following: (1) scrap loss, (2) scrap handling, (3) blank and cup, (4) washes and annealing, (5) all draws and trims, (6) bullet assembly, (7) all bullet jackets forming tools, and (8) the raw materials used to make bullet jackets. In addition, the present electroplating method reduces inventory and storage of bullet jackets.

### Summary of the invention

This invention relates to a process of making an improved small arms ammunition projectile. More specifically, the invention refers to electrodepositing a jacket onto a lead core, thereby eliminating jacket manufacture and tolerances inherent to jacket manufacturing and resulting in a low-cost accurate bullet.

It is an object of this invention to make an inexpensive small arms jacketed projectile whose performance characteristics equal or exceed conventionally-made jacketed projectiles.

It is another object of this invention to provide an economical electrodepositing method of making a jacketed small arms projectile.

A further object is to make an economical, jacketed, small arms projectile with superior mushrooming characteristics on impact.

Still another object of this invention is to provide a very accurate jacketed bullet with excellent mushrooming qualities by a mass production method.

The need for and use of jacketed bullets is well known and need not be repeated here. Although electroplating of bullets has been considered in the past, these attempts were generally unsuccessful.

Other objects and advantages of the invention will become apparent from the following description when considered in connection with the accompanying drawings.

*Brief description of the drawings*

FIGURE 1 is a cross-sectional view of a jacketed bullet incorporating the present invention.

FIGURE 2 is a view taken on line 2—2 in FIGURE 1 and shows the front end of a jacketed bullet.

FIGURE 3 is a flow diagram illustrating the various steps in the present process.

FIGURE 4 shows a magnified cross-sectional view illustrating the finger penetration of the copper jacket in the lead core which provides a strong mechanical bond.

FIGURE 5 shows a magnified cross-sectional view of a jacketed bullet which had its lead core cannelured prior to electrodepositing the copper jacket.

FIGURE 6 shows a cross-sectional view taken on line 5—5 of FIGURE 5.

FIGURE 7 shows a side view of a projectile core which is knurled and slotted prior to electrodeposition of the jacket.

FIGURE 8 shows alternate forms of recesses which can be used in place of knurling.

FIGURE 9 shows a modified sequence of forming a circumferential reinforcing bead on an electrodeposited projectile core.

*Description of the preferred embodiments*

Bullet jackets can be formed from any material that can be electroplated and any type bullet core can be used providing it can be electroplated.

The initial steps to produce an electrodeposited jacketed bullet is to cut a lead wire into slugs and then swage the slugs, thus forming profiled lead bullet cores. Obviously, other methods of forming bullet cores can also be used. As mentioned above, the profiled lead cores are the same weight and approximately the same size as the core of the ultimate jacketed bullet. The profiled lead cores are then tumbled and deburred, cleaned, rinsed, pickled, rinsed and then given a copper strike by tumbling the lead cores in a plating bath for a predetermined time until the lead cores are covered by a thin coating of copper over the entire surface of the core. This copper strike is necessary to prevent the main plating bath from becoming contaminated with lead. It has been found that when the main plating bath is contaminated with lead, the electrodeposited copper jackets tend to be brittle. The profiled lead cores entirely covered with a thin coating of copper are then continuously tumbled in the main plating bath until the required thickness of copper or other material is deposited thereon. This type of barrel plating is old and well known and it is not believed to be necessary to illustrate this step. It is, however, an important step in the process since it permits the small bullets to be continuously tumbled and plated, thus providing a uniform layer around the entire periphery of the bullet.

After the necessary thickness of copper is deposited on the bullets, the bullets are rinsed, pickled, rinsed, a corrosion inhibitor added, and the bullets dried. The plated bullets are then fed to final forming dies where they are formed to the desired configuration and dimensions and depending on the characteristics required, a front cavity and equally spaced nose cuts provided to assist mushrooming qualities of the bullets. The latter cavity and nose cuts are formed by a knockout pin which knocks the formed bullet out of the final forming dies. A proper cannelure can be formed on the plated and formed projectile as desired.

A variation in the process mentioned above may be desirable in order to satisfy certain requirements for specific bullets, etc. In other words, it may be desirable to give a certain bullet, e.g., a 6 mm. bullet, a particular mushrooming effect at a specific distance, e.g., at 100 yards. There are various procedures that can be used in this method to vary the mushrooming qualities of a bullet.

One method which is believed to be novel is to cannelure the lead core prior to electrodepositing the

copper jacket onto the profiled lead core. This method provides the forming of a controllable recess on the core into which copper deposits, thus providing a positive locking means by which the copper jacket is held onto the lead core thus aiding in preventing relative movement of the jacket and the core.

Another procedure which can be used to vary the mushrooming qualities of a bullet is to make longitudinally extending slits on the impact end of a projectile core prior to plating the projectile. Thus, transverse cannelures as well as longitudinal slits can be formed in the lead projectile core prior to plating of the projectile core. The copper is deposited over the entire surface of the core including the recesses in the cores.

After the copper is deposited over the core, a cannelure can be provided to the plated core over the cannelure previously formed in the core with the result that the deposited copper in the lead cannelure is forced inwardly to provide a deeper shoulder and a more effective locking action.

The plated projectile core with the longitudinal slits formed in the core can also be provided with unoriented slits (i.e. with the core slits) to assist in opening up the front end of the projectile upon impact.

FIGURE 1 shows a jacketed bullet 10 made according to the present invention. The bullet core 12 is formed of lead or other deformable metal and the plated jacket 14 made of a second electroplatable metal, preferably copper. A conical indent or cavity 16 and equally spaced nose cuts 18 are formed at the bullet nose to aid in mushrooming. A cannelure 20 is shown although this refinement may not be absolutely necessary to satisfactory performance.

It can be seen that the lead core 12 is entirely covered with the copper jacket 14 so that no lead is exposed. Upon impact, the cavity 16 and the nose cuts 18 assist in opening up the front end of the jacketed bullet 10 and exposing the lead core. The front end of the soft lead core 12 will then deform and peel back to form a mushroom type head having a much greater impact area than the original projectile. Since the mechanical bond between the lead core and the copper jacket (see FIGURE 3) is stronger than the lead core, the jacket does not become dislodged from the lead core, thus keeping the bullet together as a unit.

The mechanical bond between the copper jacket and lead core is best seen in FIGURE 4. This figure shows a lead core 12 and an electrodeposited copper jacket 14. The interface 22 between the lead core and the copper jacket 14 includes a plurality of recesses 24 or surface discontinuities on the outer peripheral surface of the lead core. These recesses 24 become filled with electrodeposited copper and form fingers of copper 26 penetrating into the lead, thus forming a strong bond between the two materials.

FIGURE 4 shows a cross-sectional view of a jacketed projectile made under this invention where the lead core 12 was knurled prior to having the profiled lead core plated. The figure shows an exaggerated recess 28 formed by knurling in which copper was deposited to form an abutment 30 which acts as a lock to hold the copper jacket 14 to the lead core 12.

FIGURE 5 shows a magnified cross-sectional view of the lead core 12 and the copper jacket 14 in the area where the lead core was knurled prior to plating and copper was deposited in the recesses 28 to form abutments 30. These abutments which are integrally formed with the copper jacket aid in preventing longitudinal as well as rotational movement of the jacket relative to the lead core.

FIGURE 7 shows a side view of a projectile core 32 made of lead or other suitable metal which is provided with a transverse knurl 34 and longitudinal slits 36 prior to electrodeposition of a copper or other suitable metal

jacket. After plating, a layer of copper is electrodeposited on the core and increased thicknesses are deposited in the recesses (knurling, slits, etc.) formed in the lead core.

FIGURE 8 shows various possible recesses which can be used on projectiles, either on the core or on the finished projectile.

The recesses are important, of course, to hold the electrodeposited jacket of copper onto the lead core, as well as to provide a stop for the metal jacket as it mushrooms back upon impact.

It has been found that the slits 36 or nose cuts cause cleavage of copper plate at these lines when the jacket is deposited onto the core. These cleavages weaken the jacket at these points and tend to rupture upon impact of the projectile. If the mushrooming characteristics of the projectile are not satisfied by the weakened jacket, additional slits or nose cuts can be made to the outside of the plated projectile. These outer slits need not be oriented with the slits in the core in order to be effective.

FIGURE 9 shows a sequence of the initially formed lead core 38, the plated lead core 40 and the finished bullet 42. It can be seen from this sequence that the profile of the plated lead core is changed to a greater degree than the other modifications in the forming of the plated core into the finished bullet. In this instance, the forming changed the profile of the front cylindrical portion 44 into a tapered ogival portion 46 with a reinforcing bead 48. This reinforcing bead or fold provides an excellent lock between the core and the jacket and also functions to limit the mushrooming of the projectile to the forward portion of the projectile.

The reinforcing bead 48 is stronger than the recess which would be formed by either recessing the core prior to plating or forming the recess on a tapered plated core.

The uniformity of the jacket and the mechanical bond which prevents any relative movement between the lead core and the jacket are factors which result in very substantial improvements in accuracy of the jacketed bullet.

We claim:

1. A process of making a jacketed small arms projectile comprising the following steps:

- (1) Providing a slug made of deformable and electroplatable metal;
- (2) Forming the deformable metal slug into a projectile core having a size and shape approximately the same as and a weight substantially the same as the final projectile core;
- (3) Barrel plating the deformable projectile core to electrodeposit and mechanically bond a predetermined uniform layer of a second metal on the entire exposed area of the core;
- (4) Providing slit means at one end of the jacketed projectile to assist the initiation of mushrooming deformation of jacket and core upon impact of the jacketed projectile; and
- (5) Forming the jacketed projectile into its final shape and dimensions.

2. A process as recited in claim 1 wherein recesses are provided in said deformable projectile core prior to electrodeposition thereon whereupon said recesses in the core fill up with deposited second metal thus forming a positive lock between the projectile core and the jacket.

3. A process as recited in claim 1 wherein the final forming of the jacketed projectile includes forming of an inwardly diverging cavity at the one end of the projectile jacket adjacent said slit means.

4. A process as recited in claim 1 wherein said deformable projectile core is given a thin coating of said electrodeposited second metal in a separate plating bath before being tumbled in the final plating bath where the bulk of the metal jacket is deposited.

5. A process of making a jacketed small arms projectile with predetermined mushrooming qualities comprising the following steps:

- (1) Forming a deformable metal slug into a projectile core;
- (2) Altering the deformable projectile core before plating to form recesses at desired locations thereon;
- (3) Barrel plating the altered deformable projectile core to electrodeposit a jacket of a second metal on the entire exposed area of the projectile core with increased metal thicknesses being obtained at said desired locations; and
- (4) Forming and sizing the jacketed projectile into its final shape and dimensions.

6. A process as defined in claim 5 wherein prior to the final projectile forming step, said electroplated projectiles are first provided with appropriate slit means at one end and on the outer surface of the projectile jacket to assist in initiation of mushrooming of the projectile.

7. A process of making a jacketed small arms projectile comprising the following steps:

- (1) Forming a deformable metal slug into a projectile core having a two-step predetermined profile;
- (2) Barrel plating the deformable projectile core to electrodeposit and mechanically bond a predetermined jacket of a second deformable metal on the entire exposed area of the core; and
- (3) Forming the plated projectile core to upset and change the profile thereof and provide a transverse circumferential fold about the plated projectile to act as a lock means between the projectile core and the electrodeposited jacket, the weight of the finished projectile having substantially the same weight as the plated projectile core before the final forming operation.

8. A process of making a jacketed small arms projectile comprising the following steps:

- (1) Forming a deformable metal slug into a projectile core;
- (2) Altering the deformable projectile core before plating to form recesses at desired locations thereon;
- (3) Barrel plating the altered deformable projectile core to electrodeposit a jacket of a second metal on the entire exposed area of the projectile core, said jacket being of substantially uniform thickness except that an increased metal thickness is obtained at said recesses;
- (4) Forming and sizing the plated projectile; and
- (5) Depressing said plated projectile at the area of increased jacket thickness to force the internal profile further inwardly toward the bullet axis to provide an increase in internal shoulder height.

#### References Cited

#### UNITED STATES PATENTS

2,336,143 12/1943 Werme ----- 29—1.23

RICHARD H. EANES, JR., Primary Examiner.

UNITED STATES PATENT OFFICE  
CERTIFICATE OF CORRECTION

Patent No. 3,431,612

March 11, 1968

Julius Darigo et al.

It is certified that error appears in the above identified patent and that said Letters Patent are hereby corrected as shown below:

Column 1, line 28, "3,349,722" should read -- 3,349,711 --.

Signed and sealed this 31st day of March 1970.

(SEAL)

Attest:

Edward M. Fletcher, Jr.

Attesting Officer

WILLIAM E. SCHUYLER, JR.

Commissioner of Patents